

Dec. 30, 1947.

R. P. MONSAERT, SR

2,433,620

PROCESS OF TREATING CLOTH

Filed June 28, 1944

2 Sheets-Sheet 1



Fig. 2.



INVENTOR  
Richard P. Monsaert, Sr.

BY

Gifford, Scull, & Burgess  
ATTORNEYS

Dec. 30, 1947.

R. P. MONSAERT, SR

2,433,620

PROCESS OF TREATING CLOTH

Filed June 28, 1944

2 Sheets-Sheet 2



INVENTOR.  
Richard P. Monsaert, Sr.

BY

Gofford, Kull & Burgess  
ATTORNEYS

## UNITED STATES PATENT OFFICE

2,433,620

## PROCESS OF TREATING CLOTH

Richard P. Monsaert, Sr., Paterson, N. J., assignor to United Merchants & Manufacturers, Inc., Wilmington, Del., a corporation of Delaware

Application June 28, 1944, Serial No. 542,572

4 Claims. (Cl. 195—8)

1

This invention relates to a process of treating cloth and to the cloth produced by the process. The invention will be described in its application to light suiting material containing artificial fibres, but it is of much wider application, being applicable to cloth of varied composition which is designed for the very widest uses.

Cloth made from artificial fibres such as regenerated cellulose and cellulose acetate has characteristics of coolness and light weight which fit it for use as suiting material for summer suits. The usual process of making such cloth from staple fibres is, in brief, to spin a thread from the staple fibres, size it, weave it into cloth, boil the cloth in an aqueous bath containing a size remover, boil it in a soap or other detergent solution to remove the freed particles of size and pieces of dirt, and to rinse it. The cloth so produced shows a change in dimensions, for example, a piece containing 50% regenerated cellulose and 50% cellulose acetate staple fibres in the warp and 75% regenerated cellulose and 25% cellulose acetate in the filling, when treated by the regular process shrank 5% in the warp and increased .2% in the filling, while the area was reduced from 100 to 95.2%. The weight in ounces per square yard increased very little, from 6.60 ounces per square yard to 6.62 ounces per square yard. There was no improvement in crease resistance. Such cloth wrinkles so badly, and is of such relatively light and transparent texture, that its desirable qualities are outweighed. Distinct openings, visible under a magnifying glass or even to the eye, are left between the warp and filling threads, and the threads have a glossy sheen, even when delustered, which is inferior to the matte appearance of wool. As a result, only unsatisfactory suitings have been made of this material.

Heretofore it has been proposed to overcome these disadvantages by impregnating the cloth with a solution of a synthetic resin which, upon evaporation, leaves the fibres coated with the resinous material. That treatment, although successful in its main objects, is expensive, raises the price of the treated cloth, and has certain disadvantages which need not be set forth here.

It is an object of this invention to improve the characteristics of cloth composed of or comprising regenerated cellulose and cellulose acetate.

2

Another object of the invention is to improve cloth containing other artificial fibres which are insoluble in water, and to improve cloth containing more or less cotton. Another object of the invention is to improve the crease resistance, the feel, the density, the texture, and the appearance of such types of cloth. It is another object of the invention to attain the objects of this invention without the addition of foreign substances to the cloth.

Other objects of the invention will be apparent from a reading of the specification.

The objects of the invention are accomplished generally speaking by subjecting the fabric to a tumbling and beating action in an aqueous solution of a diastatic substance such as a starch hydrolyzing agent or other size removing substance, to a tumbling and beating action in an aqueous detergent, and to a tumbling and beating action in water, the treatment being carried out preferably at an elevated temperature below that at which the fibres are adversely affected or the size remover rendered ineffective.

A particular phase of my invention concerns cloth composed of mixed regenerated cellulose and cellulose acetate fibres but the process is applicable with equal success to cloth containing many kinds of mixed fibres such as cellulose acetate and cotton, cotton and regenerated cellulose, and even to cloth composed of a single unmixed type of fibre. In some instances, a proportion of silk has been in cloth which has been successfully treated. The full advantages of the invention are obtained only on cloth made from strands composed of short fibres such as staple artificial fibres and cotton, but a few advantages of the treatment can be observed in cloth composed of continuous filaments, although the effect upon such cloth made from continuous filaments, is not equivalent to the effect of the process upon cloth made from staple fibres and the like.

My new process, as applied to the treatment of sized cloth, is carried out in a rotary machine similar in construction to that which is employed in washing, comprising generally a rotatable foraminous cylinder dipping more or less deeply into an aqueous bath. In this case, the cylinder is made reversible, going three revolutions in one direction and two in the other, and the cylinder

is interiorly provided with projecting baffles against which the cloth is beaten.

The apparatus is supplied with an adequate amount of a bath containing a size removing agent called a diastatic substance, which in the case of a starch size, may be an enzyme containing substance such as "Diastofor." The cloth is unreeed from its bolt and allowed to lie freely in the cylinder. The apparatus is then closed and the cylinder is rotated for a period of time and at a temperature sufficient to accomplish the detachment of the size from the fibres. In the case of this particular starch removing agent, a satisfactory temperature is about 140° F. and a satisfactory time of treatment is twenty minutes. Cloth sized with gelatin, glue, and sulfonated tallow, has also been successfully treated, using agents such as dilute caustic soda, soap, water, and various proprietary products.

The first bath is removed and is replaced by an aqueous detergent solution such as soap and water, which removes the dislodged sizing and the dirt which is in the cloth. The tumbling and beating action is continued in this step of the process at an elevated temperature, which may approach boiling but may satisfactorily be carried out at about 140° F. for about twenty minutes.

The detergent solution is drawn off and fresh water, preferably warm, is run in and the cloth is subjected to a tumbling and beating action in the fresh water, which removes residues of soap and the like and serves as a rinse.

In all the steps of the process the temperature used is described as warm, by which term is meant any temperature below boiling which does not damage the cloth or stop the action of the size removing agent. The treatment is carried out, frequently, until no further change in the cloth is produced by further treatment. In cases where fibres of extreme tenderness constitute a portion of the cloth, it is advisable to stop the treatment before those fibres are harmed.

It will be understood, that cloth is made of a very great variety of fibres in almost infinite percentage mixtures, and that it will be necessary for each type of cloth to receive some variation in treatment due to its particular constitution. However, the variables are simple and can be manipulated with good success by persons skilled in the art.

The invention will be further described by reference to the accompanying drawing in which—

Fig. 1 shows an elevational view of apparatus for practicing the method of the invention;

Fig. 2 shows a perspective and diagrammatic view thereof, the outer shell being shown in phantom to show the inner shell more clearly;

Fig. 3 shows a section on the line 3—3 of Fig. 2;

Fig. 4 shows a conventional staple synthetic yarn; and

Fig. 5 shows the same yarn after treatment according to the present invention, and indicates one effect which is produced by the invention.

The apparatus includes a stationary cylindrical housing or drum 1, within which is rotatably mounted a drum 2 comprising end walls 3 and 3A and a perforated cylindrical surface 4. The inner drum is divided into three compartments by diaphragms 5 and 6, each compartment being provided with a door 7 provided with a handle 7A, through which to charge the fabric to be treated.

The inner drum is mounted on trunnions 8 pass-

ing through and supported in suitable hubs or bearings 9 mounted on the end walls of the outer drum, to which trunnions are attached large gear wheels 10 which mesh with smaller gears 11, one of which in turn meshes with a pinion gear 12 mounted on a shaft 13 connected by the coupling 14 to the driving shaft 15 of a motor 16 which is so equipped that it will rotate a predetermined number of revolutions in one direction and is then reversed and rotates in the opposite direction. The specific mechanism for this reversal is well known and need not be described. The bearings 9 are supported by upright standards or brackets 20, which also support bearings 21 in which is rotatably mounted the shaft 22 to which the gears 11 are secured. The upright brackets 20 also support a horizontal platform 23, on which are mounted the motor 16 and the brackets 24, 25 carrying bearings 26, 27 in which is mounted the shaft 13 to which the pinion 12 is secured. The cylindrical surface of the outer drum has doors 18, which, in co-operation with the doors 7 on the inner drum, provide for charging the fabric and removing it. Legs 32 support the apparatus. Four bars or baffles 30 are mounted longitudinally and from one end wall 3 to the other end wall 3A of the rotatable drum. These bars may be mounted, as shown, at positions located equi-angularly about the interior circumference of the rotatable drum. The outer drum may be filled about half-full with a desired solution—as, for example, a 6% aqueous solution of any suitable diastatic preparation. Such preparations are well known in the textile industry and the specific composition thereof need not be described.

In carrying out the process with a fabric containing starch, a piece of the fabric which may have a length of 60 to 80 yards and a width of about one yard, is placed loosely in each of the compartments in the inner drum, the outer drum being about half full of the solution above mentioned. The solution is then heated to about 140° F., e. g., by means of a steam coil and the inner drum is rotated first in one direction and then in the other for about twenty minutes. During this treatment the fabric is subjected to a tumbling and beating action, the tumbling being effected by the motion of the drum and the beating being effected by the impact of the fabric on the longitudinal bars 30.

At the end of this operation the solution containing the starch hydrolytic agent is drawn off through a drain pipe, not specifically shown, and is replaced by a dilute detergent solution—e. g., one containing about 1% of soap or other detergent. The operation is then repeated for about the same period. Thereafter the fabric is rinsed in fresh water and is removed from the apparatus. It is in suitable condition for any desired subsequent treatment—e. g., bleaching, and dyeing.

The effect of the process upon one type of goods, and to some extent the nature of the goods produced by the process, can be comprehended by reference to the following table. The test was carried out on the type of goods called "Frost-point." Lot #2 of this material was divided and half left in greige and the other half was treated according to the process of this invention. In order to average the goods, a sample was taken from each end and one from the middle of each of the divisions.

Another sample of the same material called #9

was similarly divided, one half being given the regular finish and the other half left in greige.

The construction, count, thickness, weight per running yard, weight per square yard, density, and crease resistance were measured on the samples taken:

and an improvement over any cloth of similar constitution known to the prior art.

The process can be applied to unsized cloth. This treatment is carried out by soaping or treating with other detergents, and by rinsing while subjecting the cloth to the tumbling and beating

Table

|                                 | Width, inches | Warp Ends per inch | Picks per inch | Thickness in 1000's of an inch | Weight, oz.      |              | Density Grams per cm. <sup>2</sup> |
|---------------------------------|---------------|--------------------|----------------|--------------------------------|------------------|--------------|------------------------------------|
|                                 |               |                    |                |                                | Per Running Yard | Per Sq. Yard |                                    |
| <b>Piece #2 in greige:</b>      |               |                    |                |                                |                  |              |                                    |
| End.....                        | 42.3          | 58.0               | 42.7           | 20.08                          | 7.82             | 6.66         | .441                               |
| Middle.....                     | 42.3          | 58.3               | 42.7           | 19.37                          | 7.77             | 6.62         | .454                               |
| End.....                        | 42.3          | 58.0               | 43.0           | 20.06                          | 7.75             | 6.60         | .438                               |
| Average.....                    | 42.3          | 58.1               | 42.8           | 19.84                          | 7.78             | 6.63         | .445                               |
| <b>Piece #2 New Process:</b>    |               |                    |                |                                |                  |              |                                    |
| End.....                        | 39.1          | 63.0               | 46.4           | 21.66                          | 8.07             | 7.45         | .457                               |
| Middle.....                     | 39.0          | 63.2               | 46.0           | 22.03                          | 8.11             | 7.48         | .452                               |
| End.....                        | 38.9          | 63.0               | 46.2           | 21.93                          | 8.08             | 7.48         | .466                               |
| Average.....                    | 39.0          | 63.1               | 46.2           | 21.87                          | 8.09             | 7.47         | .455                               |
| <b>Piece #3 in greige:</b>      |               |                    |                |                                |                  |              |                                    |
| End.....                        | 42.4          | 58.0               | 42.5           | 20.26                          | 7.77             | 6.60         | .434                               |
| Middle.....                     | 42.4          | 57.7               | 42.7           | 20.35                          | 7.72             | 6.56         | .429                               |
| End.....                        | 42.3          | 57.7               | 43.0           | 20.46                          | 7.83             | 6.65         | .432                               |
| Average.....                    | 42.4          | 57.8               | 42.7           | 20.36                          | 7.77             | 6.60         | .432                               |
| <b>Piece #3 Regular Finish:</b> |               |                    |                |                                |                  |              |                                    |
| End.....                        | 42.1          | 58.0               | 45.8           | 19.59                          | 7.82             | 6.69         | .454                               |
| Middle.....                     | 42.6          | 57.9               | 43.8           | 19.83                          | 7.70             | 6.51         | .436                               |
| End.....                        | 42.6          | 57.8               | 45.8           | 20.15                          | 7.98             | 6.74         | .445                               |
| Average.....                    | 42.4          | 57.9               | 45.0           | 19.86                          | 7.80             | 6.62         | .445                               |

The regular finish produced a 5% dimensional change in the warp, whereas the new process produced a 7.5% change. In the filling the regular finish showed little change but the new process 40 produced a change of 7.9%. In area the new process produced a 10% greater change than the regular process. The new process produced an increase in weight of 12.5%, whereas the regular process produced an increase of only 0.3%. The crease resistance of the greige was not improved by the regular process but was materially improved by the new process.

The cloth produced by this new process is different in appearance and quality from any cloth of similar fibre content known to the prior art. When folded and crushed under a weight, this cloth does not form sharp permanent creases, but tends to resist creasing and rather to form soft full folds. The feel of the cloth is softer and more like the feel of wool than the feel of the untreated material. The density of the new cloth is greater than that of the untreated cloth and greater than that of identical cloth treated by the regular process. The texture of the cloth treated by the new process is better than the texture of the untreated cloth or of the cloth treated by the regular process. The apertures in the cloth are filled with interlaced fibres, whereas in the untreated cloth the apertures, according to the nature of the weave, are much more open. The cloth prepared according to the new process has a different appearance than any cloth of similar constitution known to the prior art. Its surface has a misty, matte appearance similar to that of good woolen cloth and apparently for a similar reason, namely, that there is a fine mist formed on the surface of the cloth by the loose and matted ends of fibres. All of these characteristics together constitute a material different from 75

action hereinbefore described. It is sometimes beneficial to include a diastatic substance in this treatment even though no sizing is present.

As many apparently widely different embodiments of this invention may be made without departing from the spirit and scope thereof, it is to be understood that it is not limited to the specific embodiments thereof except as defined in the appended claims.

What is claimed is:

1. Process of treating starch-sized fabric composed of cellulose acetate and regenerated cellulose staple fibers to remove the size and at the same time to improve its resistance to creasing which comprises subjecting the fabric to a tumbling and beating action in an aqueous bath containing a small amount of a diastatic material at about 140° F. and for a period of about 20 minutes, then subjecting the fabric to a tumbling and beating action in a warm aqueous detergent solution, thereafter subjecting said fabric to a tumbling and beating action in warm water and recovering as a result of the foregoing steps a fabric of improved resistance to creasing.

2. Process of removing the size and coincidentally improving the crease resistance of a sized, lightweight suiting fabric composed of cellulose acetate and regenerated cellulose staple fibers which comprises subjecting the fabric to a tumbling and beating action in a warm aqueous bath containing a size-removing agent until the size is detached from the fibers, then subjecting the fabric to a tumbling and beating action in a warm aqueous detergent solution, thereafter subjecting said fabric to a tumbling and beating action in warm water, and recovering as a result of the foregoing steps a fabric of improved resistance to creasing.

3. Process of simultaneously removing the

size and improving the crease resistance of a sized fabric composed of artificial staple fibers which comprises subjecting the fabric to a tumbling and beating action in a warm aqueous bath containing a size-removing agent, then subjecting the fabric to a tumbling and beating action in a warm aqueous detergent solution, thereafter subjecting said fabric to a tumbling and beating action in warm water, and recovering as a result of the foregoing steps a fabric of improved 10 resistance to creasing.

4. Process of coincidentally removing the size from and improving the crease resistance of a sized fabric composed of cellulose acetate and regenerated cellulose staple fibers which comprises 15 beating and tumbling the loose fabric in a warm aqueous solution of a diastatic size-removing agent for a time sufficient to detach the size from the fibers of the fabric, then beating and tumbling the fabric in a warm aqueous detergent solution, then beating and tumbling the fabric in 20 warm water to rinse the same, and then recov-

ering the fabric, said fabric as a result of the foregoing treatment having a greater crease resistance than the untreated fabric.

RICHARD P. MONSAERT, SR.

#### REFERENCES CITED

The following references are of record in the file of this patent:

#### UNITED STATES PATENTS

| Number    | Name      | Date           |
|-----------|-----------|----------------|
| 1,679,767 | Gminder   | Aug. 7, 1928   |
| 1,717,316 | Heberlein | June 11, 1929  |
| 1,717,992 | Melland   | June 18, 1929  |
| 1,722,171 | Bassett   | July 23, 1929  |
| 1,825,178 | Coghill   | Sept. 29, 1931 |
| 1,945,330 | Nord      | Jan. 30, 1934  |
| 1,961,608 | Ells      | June 5, 1934   |
| 1,986,945 | Schwartz  | Jan. 8, 1935   |
| 2,191,977 | Schneider | Feb. 27, 1940  |
| 2,211,841 | Voegeli   | Aug. 20, 1940  |
| 2,325,544 | Redman    | July 27, 1943  |